

## UNITED STATES PATENT OFFICE

2,662,806

## PROCESS FOR THE DYEING OF CELLULOSIC MATERIALS AND DYESTUFF PREPARATIONS SUITABLE FOR THIS PURPOSE

Karl Menzi, Henri Riati, and Jacques Wegmann,  
Basel, Switzerland, assignors to Ciba Limited,  
Basel, Switzerland, a Swiss firmNo Drawing. Application July 20, 1950,  
Serial No. 175,014Claims priority, application Switzerland  
July 29, 1949

14 Claims. (Cl. 8—42)

1

The present invention is based on the observation that cellulosic materials are dyed in a valuable manner when the dyeing is carried out with a metal compound, difficultly soluble per se, of a direct dyeing azo dyestuff which contains in complex combination one of the metals with the atomic numbers 27 to 29, or with a mixture for the formation thereof, in the presence of an aliphatic base free from acid groups, which contains at least one basic nitrogen atom and at least one hydroxyl group separated from the basic nitrogen atom by two carbon atoms, which base is solid and water-soluble.

The metal compounds which are difficultly soluble in water per se contain in complex combination one of the metals with the atomic numbers 27 to 29, that is to say, in the order of increasing importance, cobalt, nickel and copper. Especially valuable results are obtained with such azo dyestuffs containing copper as in the metal-free condition are still soluble in water and suitable for the dyeing of cellulosic materials, but which in the form of copper compounds are difficultly soluble in water and on account of this property are not of good suitability for dyeing, at all events when it is not intended to dye from a suspension, which method as a rule yields unsatisfactory results. In the present case those complex metal compounds which give colloidal solutions in water are also to be considered as difficultly soluble. It is the result of experience that these metal compounds are also unsuitable per se for dyeing on account of their very poor capacity for drawing onto the fiber.

The difficultly water-soluble dyestuffs to be employed according to the present process, may for example be metal complexes of dyestuffs with o-hydroxy carboxylic acid groupings, as are present among others in salicylic acid. In this connection there should also be mentioned metal complexes of dyestuffs with the atom grouping



As especially advantageous have proved among others metal compounds of o:o'-dihydroxyazo dyestuffs, that is to say from dyestuffs which contain the atom grouping



Also among the metal compounds of o:o'-dihydroxyazo dyestuffs the copper compounds are chiefly of value. These contain the atom grouping which is usually illustrated by the formula



10 at least once in the molecule. They can contain the atom grouping for example twice and in the following form



15 The copper compounds of such constitution which are difficultly soluble to insoluble in water can be produced by customary methods known especially for the production of water-soluble copper compounds, by treatment with agents providing copper of the corresponding metal-free azo dyestuffs which contain the atom grouping



20 In the case of azo dyestuffs with the last-mentioned grouping the treatment with agents providing copper should be carried out in such a manner that the copper complex formation takes place with splitting off of the —O-alkyl group.

25 In some cases this takes place also with dyestuffs which yield difficultly soluble copper compounds, by heating with copper tetrammine compounds of ammonia in an alkaline medium for a prolonged period. Particularly effective is however in this case the application of the process of U. S. Patent application Serial No. 778,734 (now U. S. Patent No. 2,536,957).

30 In general it is advantageous to employ or produce the complex metal compounds for the dyestuff preparations in such a condition that their ionogenic salt-forming groups, that is to say especially sulfonic acid and carboxyl groups (insofar as the latter are not used in the complex formation) exist in the form of metal salts, for example alkali metal salts and not as free acid groups or ammonium salts.

35 Instead of the complex metal compounds there can also be used in the present process the mixtures used in the formation thereof. It is thus 40 possible for example to employ a dyestuff free

## 3

from complex-forming metal, suitably in the form of an alkali salt, in combination with the necessary quantity of an agent providing metal. As agents providing metal there are also concerned in this case the compounds known per se which are normally used for the production of complex metal compounds. When as agents providing metal simply constituted metal salts are employed, as for example sulfates, nitrates or acetates, it is in general advantageous to add to the 10 dyebaths in addition to the metal salts further suitable additions which during the dyeing are capable of dispersing any metal hydroxide produced. As an example of such an addition may be mentioned the sodium salt of  $N$ -methyl- $\mu$ -heptadecyl-benzimidazole sulfonic acid.

There may be used with advantage as agents providing metal such compounds of complex-forming metals as contain the metal in complex combination in the anion. In any case the complex formers should not possess the property of withdrawing metal from the complex metal compounds of dyestuffs under the working conditions concerned. As examples of useful complex formers may be mentioned aliphatic hydroxy carboxylic acids such as glycollic acid, lactic acid,  $\beta$ -hydroxypropionic acid,  $\beta$ -hydroxybutyric acid, tartaric acid and citric acid.

It is to be recommended to employ a certain 30 excess of the agent providing metal over the theoretically necessary quantity.

According to the present invention the dyeing with the complex metal compounds of the above described composition takes place in the presence of an aliphatic base. This base contains at least 35 one basic nitrogen atom and is solid, that is to say its melting point lies above the temperatures at which the preparations are normally stored; it is therefore higher than 40° C. The base is in addition water-soluble and free from acid groups such as sulfonic acid groups and carboxyl groups; on the other hand it contains at least one hydroxyl group, which is separated from the basic 40 nitrogen atom by two carbon atoms. Of particularly good suitability are the bases of the composition



in which  $R_1$  indicates a hydrogen atom, an alkyl group with at the most three carbon atoms or a hydroxymethyl group,  $R_2$  a hydrogen atom or a methyl group and  $n$  a whole number which is at the most 4 but preferably 2.

As examples may be mentioned the bases of the following composition:



M. P. 93 to 94° C.



M. P. 136 to 139° C.



M. P. 177 to 181° C.

## DR. K. H. WILHELM

## 4



M. P. 154 to 157° C.

These bases can be produced for example in an analogous manner to that described in German Patent No. 635,904 by condensation of hydroxyalkylamines with dihalogenalkyls.

The quantity proportion between the complex metal compound or the mixture for the formation thereof and the organic base is in the present process with advantage so selected that a considerable excess of the base is present, that is to say for one atom of complex-bound metal several molecules of base are present, for example more than two or a still higher number.

The present invention renders it possible to dye on cellulosic fibers directly in a single bath and a single stage process, as complex metal compounds, without adding further materials to the dyebath apart from the customary auxiliary agents in the direct dyeing process such as sodium sulfate and/or sodium carbonate, direct dyeing azo dyestuffs of which the metal complexes are per se difficultly soluble in water and which therefore are unsuitable for dyeing as complex metal compounds, for which reason they are usually employed in the metal-free condition and are only converted into the metal compounds when they are at least for the most part fixed on the fiber. The bath ratio, that is to say the ratio of the quantity of the material to be dyed to the quantity of the dye liquor can in this case be varied within wide limits and can be suited to a far-reaching extent to the requirements of practice. If desired, as is customary in practice, prior to the preparation of the dyebaths, concentrated solutions, so-called stock solutions, can be formed with the base and the complex metal compound or with the base, the metal-free dyestuff and the agent providing metal, which solutions are then diluted to the larger volumes necessary for dyeing.

According to the present process there are obtained in this manner as a rule dyeings which as regards color strength, purity of the dye shade and fastness properties are at least equivalent to and in part are superior to those dyeings which are obtained when a corresponding quantity of dyestuffs free from metals and bases is dyed by the after-metallisation process.

In certain cases it may further be of advantage to after-treat dyeings obtainable according to the present process with such agents as increase 60 their wet fastness properties. This after-treatment can also take place in the presence of agents providing copper. As products which improve the wet fastness properties of dyeing there may be mentioned among others the products of the 65 action of formaldehyde on compounds such as cyanamide, dicyandiamide, dicyandiamidine, melamine and so on. Such after-treating agents are also concerned, in the production of which no formaldehyde is used. The application of after-treating agents containing copper is to be 70 recommended especially when there are indications that during the dyeing a more or less far-reaching de-coppering takes place.

Instead of bringing together the base and the 75 complex metal compound or the base, the metal-

free dyestuff and the agent providing metal, in the dyebath or in one of the previously mentioned, so-called stock solutions, it is to be recommended in general to work up the materials concerned to dry or if desired paste preparations. These new dyestuff preparations, suitable for carrying out the initially described dyeing process, accordingly contain a metal compound of a direct dyeing azo dyestuff, which compound per se is difficultly soluble and which contains in complex combination one of the metals with the atomic numbers 27 to 29, or a mixture for the formation thereof, and also contain an aliphatic base free from acid groups, which contains at least one basic nitrogen atom and at least one hydroxyl group separated from the basic nitrogen atom by two carbon atoms and which base is solid, water-soluble and capable of imparting solubility to the complex metal compounds.

The dyestuff preparations are suitably produced by mixing the individual required components, for example in the dry state. They can however also be produced in the moist condition, for example in paste form or by combination of solutions or by association of moist or dissolved components of the mixture with dry components of the mixture followed if desired by drying. In the production of the dyestuff preparations by the wet method it is possible that preparations may be obtained in which at least a portion of the complex metal compound of the dyestuff has undergone chemical combination with the base. The preparations can also be subjected to admixture with further substances, such as urea or water-soluble carbohydrates, for example saccharose. On the other hand it is in general less to be recommended to incorporate in large quantities electrolytes such as sodium sulfate or sodium chloride.

The following examples illustrate the invention, the parts and percentages being by weight unless otherwise stated and the relation between parts by weight and parts by volume being the same as that between the kilogram and the liter. Where the production of dyebaths and stock solutions is described, as "water" preferably so-called condensed water (distilled water recovered from live steam) is to be employed.

#### Example 1

2 parts of 1:2-di-( $\beta$ -hydroxyethylamino)-ethane are mixed with 1 part of the copper compound of the dyestuff which is obtained by phosgenation of 1 mol of 4-amino-4'-hydroxy-3'-carboxy-1:1'-azobenzene and 1 mol of the condensation product of 4-amino-2-methyl-5-methoxy-4'-hydroxy-3'-carboxy-1:1'-azobenzene-5'-sulfonic acid with 4-nitrobenzoyl chloride of which product the nitro group has been reduced to the amine.

With this dyestuff preparation cotton can be dyed for example in the following manner:

3 parts of the dyestuff preparation are covered with 200 parts of hot water and the whole brought to the boil. From the stock solution obtained there is prepared by dilution with water to 3000 parts by volume and addition of 2 parts of anhydrous sodium carbonate, a dyebath into which at about 60° C. are entered 100 parts of previously wetted cotton. Within  $\frac{1}{4}$  hour the temperature is raised to boiling and it is maintained for one hour at boiling temperature, during which after 5 minutes and after 20 minutes boiling in each case 20 parts of crystalline sodium sulfate are added.

After rinsing and drying of the cotton a yellow 75 parts of crystalline sodium sulfate are added.

dyeing results of good fastness to light and very good fastness to washing.

The same result is obtained when the 1:2-di( $\beta$ -hydroxy-ethylamino)-ethane is replaced by the same quantity of any of the products which are obtained by condensation in each case of 1 mol of 1:2-dichlorethane with 2 mols of isopropanolamine, 1-hydroxy-2-amino-2-methylpropane or 1:3-dihydroxy-2-amino-2-methylpropane.

Similar dyeings are obtained when the copper compound is replaced by the nickel or cobalt compound of the dyestuff initially mentioned.

#### Example 2

Equal parts are mixed of 1:2-di-( $\beta$ -hydroxy-ethylamino)-ethane and the copper compound of the dyestuff which is obtained as follows:

1 mol of the monoazo dyestuff from diazotized 1-amino-4-hydroxy-5-carboxybenzene and 1-aminonaphthalene-7-sulfonic acid is diazotized and coupled with 1 mol of 1-aminonaphthalene. The amino compound obtained is again diazotized and coupled in an alkaline medium with 1 mol of 2-amino-5-hydroxynaphthalene-7-sulfonic acid.

With this dyestuff preparation cotton can be dyed for example as follows:

2 parts of the dyestuff preparation are covered with 200 parts of water and the whole brought to the boil. From this stock solution is prepared by dilution to 3000 parts by volume and addition of 2 parts of anhydrous sodium carbonate, a dyebath into which at about 60° C. are entered 100 parts of previously wetted cotton. Within  $\frac{1}{4}$  hour the temperature is raised to boiling and the whole is maintained for 1 hour at boiling temperature during which after 5 minutes and after 20 minutes boiling in each case 20 parts of crystalline sodium sulfate are added. The dyeing is rinsed in the cold, in which operation there is advantageously added to the final rinsing bath 1 part of the condensation product which is obtained when dicyandiamidine is heated with 4 times the quantity of 30 per cent. commercial formaldehyde for about 10 minutes to 100° C. and the dyeing is allowed to remain in this bath for about 5 minutes.

A blue dyeing results of excellent fastness to light and washing.

By employing instead of 1:2-di-( $\beta$ -hydroxy-ethylamino)-ethane the bases mentioned in paragraph 5 of Example 1, equal results are obtained.

#### Example 3

Equal parts are mixed of 1:2-di-( $\beta$ -hydroxy-ethylamino)-ethane and the copper compound of the dyestuff which is obtained as follows:

1 mol of 1-(4'-amino-1:1'-diphenyl-4)-3-methyl-pyrazolone-(5) is converted by means of phosgene into the symmetrical urea derivative and the latter is coupled with 1 mol of diazotized 1-amino-2-carboxybenzene-4-sulfonic acid.

With this dyestuff preparation cotton can be dyed for example as follows:

3 parts of the dyestuff preparation are covered with 200 parts of hot water and the whole brought to the boil. From the stock solution obtained there is prepared by dilution with water to 3000 parts by volume and addition of 2 parts of anhydrous sodium carbonate, a dyebath into which at about 60° C. are entered 100 parts of previously wetted cotton. Within  $\frac{1}{4}$  hour the temperature is raised to boiling and the whole is maintained for 1 hour at boiling temperature during which after 5 minutes and after 20 minutes in each case 20 parts of crystalline sodium sulfate are added.

After rinsing and drying of the cotton a yellow dyeing results of good fastness to light and washing.

*Example 4*

2 parts of 1:2-di-( $\beta$ -hydroxyethylamino)-ethane, 3 parts of saccharose and 1 part of the copper compound of the dyestuff from 1 mol of tetrazotized 4:4'-diamino-3:3'-dihydroxy-1:1'-diphenyl and 2 mol of 2-amino-5-hydroxynaphthalene-7-sulfonic acid, are mixed together.

With this dyestuff preparation cotton can be dyed for example as follows:



2 parts of the dyestuff preparation are covered with 200 parts of water and the whole brought to the boil. From the stock solution obtained there is prepared by dilution with 2800 parts of water and addition of 2 parts of anhydrous sodium carbonate, a dyebath into which at about 60° C. are entered 100 parts of previously wetted cotton. Within  $\frac{1}{4}$  hour the temperature is raised to boiling and the whole is maintained for 1 hour at boiling temperature during which after 5 minutes and after 20 minutes in each case 20 parts of crystalline sodium sulfate are added.

After rinsing and drying of the cotton a blue dyeing is produced of excellent fastness to light and washing.

Prior to drying the dyeing can be further treated in a bath ratio of 1:30 for  $\frac{1}{2}$  hour at ordinary temperature with 4 per cent of a preparation containing per 100 parts 32 parts of a

sodium carbonate, a dyebath into which at about 60° C. are entered 100 parts of previously wetted cotton. Within  $\frac{1}{4}$  hour the temperature is raised to boiling and the whole is maintained for 1 hour at boiling temperature during which after 5 minutes and after 20 minutes boiling in each case 20 parts of crystalline sodium sulfate are added.

After rinsing and drying of the cotton a grey dyeing results of very good fastness to light and washing.

*Example 6*

2 parts of the dyestuff of the formula



condensation product from dicyandiamidine and formaldehyde, 11 parts of copper acetate, 31 parts of sodium carbonate and 18 parts of ammonium chloride. The dyeing thus treated exhibits a still further improved fastness to washing.

*Example 5*

There are mixed together 2 parts of 1:2-di-( $\beta$ -hydroxyethylamino)-ethane with 1 part of the copper compound of the dyestuff which is obtained by careful reduction with glucose in an alkaline medium of the disazo dyestuff of the following constitution:



With this dyestuff preparation cotton can be dyed for example as follows:

2 parts of the dyestuff preparation are covered with 200 parts of hot water and the whole brought to the boil. From this stock solution there is prepared by dilution with water to 3000 parts by volume and addition of 2 parts of anhydrous so-

are intimately ground with 4 parts of 1:2-di-( $\beta$ -hydroxyethylamino)-ethane and 1 part of sodium copper tartrate.

3 parts of this preparation are dissolved in 200 parts of hot water and added to a dyebath of 2800 parts of water and 2 parts of anhydrous sodium carbonate. At about 60° C. are entered 100 parts of previously wetted cotton and the temperature is raised to boiling within  $\frac{1}{4}$  hour. The bath is maintained for 1 hour at boiling temperature during which after 5 minutes and after 20 minutes in each case 20 parts of crystalline sodium sulfate are added. After this time the dyebath is substantially exhausted. The cotton is rinsed, hydro-extracted and dried. The resulting brown dyeing possesses a good fastness to washing and an excellent fastness to light.

By using instead of the above dyestuff 2 parts of the dyestuff of the formula



a preparation is obtained which dyes cotton in navy blue shades fast to washing and light.

What we claim is:

1. Process for dyeing cellulosic materials which comprises carrying out the dyeing with a metal compound difficultly soluble per se of a direct dyeing azo dyestuff which contains in complex union one of the metals with the atomic numbers 27 to 29 in the presence of a solid base of the composition



wherein  $R_1$  stands for a member selected from the group consisting of a hydrogen atom, an alkyl group with at the most three carbon atoms and a hydroxymethyl group,  $R_2$  stands for a member selected from the group consisting of a hydrogen atom and a methyl group and  $n$  represents a whole number up to 4.

2. Process for dyeing cellulosic materials which comprises carrying out the dyeing with a metal compound difficultly soluble per se of a direct dyeing azo dyestuff which contains in complex union one of the metals with the atomic num-

9. Process for dyeing cellulosic materials which comprises carrying out the dyeing with the base corresponding to the formula



3. Process for dyeing cellulosic materials which



comprises carrying out the dyeing with a complex copper compound difficultly soluble per se of a direct dyeing azo dyestuff in the presence of the base corresponding to the formula



4. Process for dyeing cellulosic materials which



comprises carrying out the dyeing with the complex copper compound of the dyestuff corresponding to the formula

30

7. Process for dyeing cellulosic materials which comprises carrying out the dyeing with the complex copper compound of the dyestuff corresponding to the formula



in the presence of the base corresponding to the formula



8. Process for dyeing cellulosic materials which comprises carrying out the dyeing with the dyestuff of the formula



in the presence of sodium copper tartrate and of the base corresponding to the formula



in the presence of the base corresponding to the formula



5. Process for dyeing cellulosic materials which comprises carrying out the dyeing with the complex copper compound of the dyestuff corresponding to the formula

45

9. A dyebath containing a metal compound difficultly soluble per se of a direct dyeing azo dyestuff which contains in complex union one of the metals with the atomic numbers 27 to 29 and also containing a solid base of the composition



R<sub>1</sub>

wherein R<sub>1</sub> stands for a member selected from



in the presence of the base corresponding to the formula



6. Process for dyeing cellulosic materials which comprises carrying out the dyeing with the complex copper compound of the dyestuff corresponding to the formula

65



in the presence of the base corresponding to the formula



10. A dyebath containing a metal compound difficultly soluble per se of a direct dyeing azo dyestuff which contains in complex union one of the metals with the atomic numbers 27 to 29

11

and also containing the base corresponding to the formula



11. A dyebath containing a complex copper compound difficultly soluble per se of a direct dyeing azo dyestuff and also containing the base corresponding to the formula



12. A dyestuff preparation containing a metal compound difficultly soluble per se of a direct dyeing azo dyestuff which contains in complex union one of the metals with the atomic numbers 27 to 29 and also containing the base corresponding to the formula



10

20

12

atom and a methyl group and  $n$  represents a whole number up to 4.

13. A dyestuff preparation containing a metal compound difficultly soluble per se of a direct dyeing azo dyestuff which contains in complex union one of the metals with the atomic numbers 27 to 29 and also containing the base corresponding to the formula



14. A dyestuff preparation containing a complex copper compound difficultly soluble per se of a direct dyeing azo dyestuff and also containing the base corresponding to the formula



KARL MENZI.  
HENRI RIAT.  
JACQUES WEGMANN.

## References Cited in the file of this patent

## UNITED STATES PATENTS

| Number    | Name   | Date          |
|-----------|--------|---------------|
| 2,092,429 | Straub | Sept. 7, 1937 |